# EUROPEAN PATENT SPECIFICATION

(11) **EP 0 027 460 B1**
(45) Date of publication and mention of the grant of the patent: **01.08.1984**
(21) Application number: 80900936.8
(22) Date of filing: 24.04.1980
(51) Int. Cl.: G03C 1/40, G03C 7/00, G03C 5/54

(54) **Diffusion transfer film unit and color process**
Diffusionsübertragungsfilmeinheit und Farbverfahren
Film unitaire pour la photographie par diffusion-transfert et procédé en couleurs

(30) Priority: 24.04.1979 US 32954
(43) Date of publication of application: 29.04.1981
(73) Proprietor: POLAROID CORPORATION, Cambridge, Massachusetts 02139 (US)
(72) Inventor: LAMBERT, Ronald F., Wayland, MA 01778 (US)
(74) Representative: Reitzner, Bruno, Dr.
(86) International application number: US8000457
(87) International publication number: WO8002331

## Description

This invention relates to diffusion transfer photography

According to US-A-2,983,606, issued May 9, 1961 to Howard G. Rogers, a photosensitive . element containing a dye developer and a silver halide emulsion is photo-exposed and a processing composition applied thereto, for example, by immersion, coating, spraying, flowing, etc., in the dark. The exposed photosensitive element is superposed prior to, during, or after the processing composition is applied, on a second sheet-like element which may be utilized an an image-receiving element. In a preferred embodiment, the processing composition is applied to the exposed photosensitive element in a substantially uniform layer as the photosensitive element is brought into superposed relationship with an image-receiving layer carried by said second sheet-like element. The processing composition permeates the emulsion to initiate development of the latent image contained therein. The dye developer is immobilized or precipitated in exposed areas as a consequence of the development of the latent image. This immobilisation is apparently, at least in part, due to a .change in the solubility characteristics of the dye developer upon oxidation and especially as regards its solubility in alkaline solutions. It may also be due in part to a tanning effect on the emulsion by oxidized developing agent, and in part to a localized exhaustion of alkali as a result of development. In unexposed and partially exposed areas of the emulsion, the dye developer is unreacted and diffusible and thus provides an imagewise distribution of unoxidized dye developer, diffusible in the processing composition, as a function of the point-to-point degree of exposure of the silver halide emulsion. At least part of this imagewise distribution of unoxidized dye developer is transferred, by imbibition, to the superposed image-receiving layer, said transfer substantially excluding oxidizing dye developer. The image-receiving layer receives a depthwise diffusion, from the developed emulsion, of unoxidized dye developer without appreciably disturbing the imagewise distribution thereof to provide a reversed or positive color image of the developed image. The image-receiving element may contain agents adapted to mordant or otherwise fix the diffused, unoxidized dye developer. In a preferred embodiment of said US-A-2,983,606 and in certain commercial applications thereof, the desired positive image is revealed by separating the image-receiving element from the photosensitive element at the end of a suitable imbibition period. Alternatively, as also disclosed in said US-A-2,983,606, the image-receiving layer need not be separated from its superposed contact with the photosensitive element, subsequent to transfer image formation, if the support for the image-receiving layer, as well as any other layers intermediate said support and image-receiving layer, is transparent and a processing composition containing a substance, e.g. a white pigment, effective to mast the developed silver halide emulsion or emulsions, is applied between the image-receiving layer and said silver halide emulsion or emulsions.

Dye developers, as noted in said US-A-2,983,606, are compounds which contain, in the same molecule, both the chromophoric system of a dye and also a silver halide developing function. By "a silver halide developing function" is meant a grouping adapted to develop exposed silver halide. A preferred silver halide development function is a hydroquinonyl group. In general, the development function includes a benzenoid developing function, that is, an aromatic developing group which forms quinonoid or quinone substances when oxidized.

Multicolor images may be obtained using dye developers in diffusion transfer processes by several techniques. One such technique contemplates obtaining multicolor transfer images utilizing dye developers by employment of an integral multilayer photosensitive element, such as is disclosed in the aforementioned US-A-2,983,606 and in US-A-3,345,163 issued October 3, 1967 to Edwin H. Land and Howard G. Rogers, wherein at least two selectively sensitized photosensitive strata, superposed on a single support, are processed, simultaneously and without separation, with a single common image-receiving layer. A suitable arrangement of this type comprises a support carrying a red-sensitive silver halide emulsion stratum, a green-sensitive silver halide emulsion stratum and a blue-sensitive silver halide emulsion stratum, said emulsions having associated therewith, respectively, for example, a cyan dye developer, a magenta dye developer and a yellow dye developer. The dye developer may be utilized in the silver halide emulsion stratum, for example in the form of particles, or it may be disposed in a stratum behind the appropriate silver halide emulsion strata. Each set of silver halide emulsion and associated dye developer strata may be separated from other sets by suitable interlayers, for example, by a layer of stratum of gelatin or polyvinyl alcohol. In certain instances, it may be desired to incorporate a yellow filter in front of the green-sensitive emulsion and such yellow filter may be incorporated in an interlayer. However, where desirable, a yellow dye developer of the appropriate spectral characteristics and present in a state capable of functioning as a yellow filter may be so employed and a separate yellow filter omitted.

Particularly useful products for obtaining multicolor dye developer images are disclosed in US-A-3,415,644 issued December 10, 1968 to Edwin H. Land. This patent discloses photographic products and processes wherein a photosensitive element and an image-receiving element are maintained in fixed relationship prior to exposure, and this relationship is maintained as a laminate after processing and image formation. In these products, the final image is viewed through a transparent (support) element against a light-reflecting, i.e., white background. Photoexposure is made through said transparent element and application of the processing composition provides a layer of light-reflecting material to provide a white background. The light-reflecting material (referred to in said patent as an "opacifying agent") is preferably titanium dioxide, and it also performs an opacifying function, i.e., it is effective to mask the developed silver halide emulsions so that the transfer image may be viewed without interference therefrom, and it also acts to protect the photoexposed silver halide emulsions from post-exposure fogging by light passing through said transparent layer if the photoexposed film unit is removed from the camera before image-formation js completed. - - - t

US-A-3,647,437, issued March 7, 1972 to Edwin H. Land, is concerned with improvements in products and processes disclosed in said US-A-3,41 5,644, and discloses the provision of light-absorbing materials to permit such processes to be performed, outside of the camera in which photoexposure is effected, under much more intense ambient light conditions. A light-absorbing material or reagent, preferably a pH-sensitive phthalein dye, is provided so positioned and/or constituted as not to interfere with photoexposure but so positioned between the photoexposed silver halide emulsions and the transparent support during processing after photoexposure as to absorb light which otherwise might fog the photoexposed emulsions. Furthermore, the light-absorbing material is so positioned and/or constituted after processing as not to interfere with viewing the desired image shortly after said image has been formed. In the preferred embodiments, the light-absorbing material, also sometimes referred to as an optical filter agent, is initially contained in the processing composition together with a light-reflecting material, e.g., titanium dioxide. The concentration of the light-absorbing dye is selected to provide the light transmission opacity required to perform the particular process under the selected light conditions.

In a particularly useful embodiment, the light-absorbing dye is highly colored at the pH of the processing composition, e.g., 13-14, but is substantially non-absorbing of visible light at a lower pH, e.g., less than 10-12. This pH reduction may be effected by an acid-reacting reagent appropriately positioned in the film unit, e.g., in a layer between the transparent support and the image-receiving layer.

The dye developers are preferably selected for their ability to provide colors that are useful in carrying out subtractive color photography, that is, the previously mentioned cyan, magenta and yellow. The dye developers employed may be incorporated in the respective silver halide emulsion or, in the preferred embodiment, in a separate layer behind the respective silver halide emulsion, and such a layer of dye developer may be applied by use of a coating solution containing the respective dye developer distributed, in a concentration calculated to give the desired coverage of dye developer per unit area, in a film-forming natural, or synthetic, polymer, for example, gelatin, polyvinyl alcohol, and the like, adapted to be permeated by the processing composition.

US-A-33 53 956 and US-A-33 77 166 disclose diffusion transfer color processes and film units therefor, of the type using dye developers. These known film units contain imidazole or substituted imidazoles as development improvers. The imidazole derivatives used as development improvers all contain an imino nitrogen atom. Their main function is to produce a glossy transfer image and to improve blue contrast, respectively. However, nothing is said or indicated about the improvement of the transfer rates of unoxidized dye developers without adverse effects on minimum density.

US-A-38 08 003 relates to the use of certain substituted imidazoles to increase the speed of development of an exposed gelatino-silver halide photographic light-sensitive material. The general formula includes four substituents Rᵢ to R₄ which are selected from the group consisting of a hydrogen atom, an alkyl group, a hydroxy alkyl group and an alkenyl group, and wherein at least one of R, to R₄ is selected from the group consisting of an alkyl group, a hydroxy alkyl group and an alkenyl group. Only if Rᵢ is a substituent other than hydrogen, one would arrive at one of the species contemplated by the present invention. However, there is no disclosure that would teach the selection of such compounds to obtain the improvement of the transfer rates of unoxidized dye developer without adverse effect on minimum density. There is no clear teaching of the use of imidazoles in color diffusion transfer in general, much less in color diffusion transfer systems employing dye developers. Speeding up development in the sense of this prior publication refers to how quickly the exposed silver halide grains containing the latent image can be developed or reduced to image silver. On the other hand, transfer of dye developers from the photosensitive element to the receiving layer has nothing to do with development. The dye developers are initially soluble and diffusible in the developer liquid, and the speed of the their transfer will not depend upon how fast the silver halide grains are developed.

It has now been found that desirable improvements may be obtained in dye developer color transfer processes if processing is effected in the presence of specifically selected diazole or diazine derivatives. Accordingly, the invention relates to a diffusion transfer film unit comprising a photosensitive element comprising a support carrying at least one photosensitive silver halide emulsion layer, each said silver halide emulsion layer having associated therewith a dye developer; an aqueous alkaline processing composition; an image-receiving layer in superposed or superposable relationship with said silver halide emulsion layer(s); characterized in that said film unit includes a 5- or 6-membered aromatic unsaturated heterocyclic diazole or diazine, respectively, free of imino nitrogen atoms, said diazole or diazine being a liquid at room temperature.

These heterocyclic diazoles and diazines, respectively, may be said to be "aromatic" in that the 5- membered heterocyclic diazoles contain two double bonds and the 6-membered heterocyclic diazines contain three double bonds. The nitrogen atoms may be adjacent or separated by one or two carbon atoms. Substituents on the ring carbons or nitrogens may include 1 to 2 carbon atoms. Examples of 5-and 6-membered unsaturated heterocyclic diazoles found useful in accordance with this invention include:

That these diazoles would be effective in this manner could not have been predicted, since such closely related compounds as the following compounds did not exhibit the same beneficial properties:

While the reason why 1-methyl-imidazole should behave so differently from, e.g., imidazole or 2-methylimidazole is not fully understood it is believed that the absence of an imino nitrogen able to form an anion in alkaline solution is in some manner responsible for the different behavior. 1-benzyl-imidazole, on the other hand is a solid at room temperature.

Further embodiments of the present invention are recited in the subclaims.

The following examples are given to illustrate the invention and are not intended to be limiting. All parts and percentages are by weight unless otherwise stated.

### Example 1

A multicolor photosensitive element using, as the cyan, magenta and yellow dye developers was prepared by coating a gelatin-subcoated 0,1 mm opaque polyethylene terphthalate film base with the following layers:
1. a layer of cyan dye developer dispersed in gelatin and coated at a coverage of about 742 mg/m² of dye and about 269 mg/m² of gelatin, and also containing about 269 mg/m² of 2-phenyl benzimidazole, and about 68 mg/m² of 4'-methylphenyl hydroquinone;
2. a red-sensitive gelatino silver iodobromide emulsion coated at a coverage of about 1291 mg/m² of silver and about 775 mg/m² of gelatin;
3. a layer of a 60-30-4-6 copolymer of butylacrylate, diacetone acrylamide, styrene and methacrylic acid and polyacrylamide coated at a coverage of about 2505 mg/m² of the copolymer and about 77.5 mg7m² of polyacrylamide;
4. a layer of magenta dye developer dispersed in gelatin and coated at a coverage of about 646 mg/m² of dye and about 452 mg/m² of gelatin, and also containing about 226 mg/m² of 2-phenyl benzimidazole;
5. a green-sensitive gelatino silver iodobromide emulsion coated at a coverage of about 796 mg/m² of silver and about 387 mg/m² of gelatin;
6. a layer containing the copolymer referred to above in layer 3 and polyacrylamide coated at a coverage of about 1367 mg/m² of copolymer and about 87 mg/m² of polyacrylamide, and about 71 mg/m² of succinaldehyde;
7. a layer of yellow dye developer dispersed in genatin and coated at a coverage of about 968 mg/m² of dye and about 452 mg/m² of gelatin, and also containing about 204 mg/m² of 2-phenyl benzimidazole;
8. a blue-sensitive gelatino silver iodobromide emulsion layer including 4'-methylphenyl hydroquinone coated at a coverage of about 1280 mg/m² of silver, about 667 mg/m² of gelatin and about 204 mg/m² of 4'-methylphenyl hydroquinone; and
9. a layer of gelatin coated at a coverage of about 484 mg/m² of gelatin and containing about 43 mg/m^{l} of carbon black.

A transparent 0.1 mm polyethylene terephthalate film base was coated, in succession, with the following layers to form an image-receiving component:
1. as a polymeric acid layer, a mixture of a partial butyl ester of polyethylene/maleic anhydride copolymer and polyvinyl butyral at a ratio of about 9:1 at a coverage of about 26900 mg/m²;
2. a timing layer containing about a 45:0.7 ratio of a 60-30-4-6 copolymer of butylacrylate, diacetone acrylamide, styrene and methacrylic acid and polyvinyl alcohol at a coverage of about 484 mg/m²; and
3. an image-receiving layer containing a'2:1:1 mixture of polyvinyl alcohol, poly-4-vinyl pyridine and a graft copolymer of 4'-vinyl pyridine and vinylbenzyl trimethyl ammonium chloride on hydroxyethyl cellulose (2.2:1:2.2 ratio) at a coverage of about 3328 mg/m².

The photosensitive component was photoexposed and then taped to one end of the image-receiving component with a rupturable container retaining an aqueous alkaline processing solution fixedly mounted on the leading edge of each of the components, by pressure-sensitive tapes to make a film unit, so that, upon application of compressive pressure to the container to rupture the container's marginal seal, its contents would be distributed between the image-receiving layer and the gelatin overcoat of the photosensitive component. The aqueous alkaline processing composition comprised:

A layer approximately 0.076 mm thick of the processing composition was distributed by passing the film unit between a pair of pressure-applying rolls and into a lighted area. The resulting laminate was maintained intact to provide a multicolor integral negative-positive reflection print.

The above procedure was repeated except that 1-methyl imidazole was added to the processing composition at a concentration of about 1% by weight.

The maximum and minimum reflection densities of the neutral column of the control and test. images were measured at intervals of time after the processing composition was applied, and the following results were obtained.

It will be apparent that the inclusion of the 1-methyl imidazole resulted in faster dye transfer, particularly of the magenta dye developer. It will also be noted that the final minimum densities were substantially unchanged. (The decrease in minimum densities was due to the fact that early density readings necessarily included density contributed by the phthalein opacifying dyes prior to their decolorization.)

Good results with N-methyl imidazole also were obtained with the same film unit using higher concentrations, e.g., 1.75% and 2.5%. The substitution of 1,2-dimethyl imidazole for 1-methyl imidazole in the above experiment also gave increased transfer rates of unoxidized dye developer without adverse effect upon minimum density.

### Example 2

A photosensitive element was prepared similar to the one described in Example 1, using the same cyan and yellow dye developers and the following magenta dye developer: The coverages of the cyan, magenta and yellow dye developers, respectively, were on the order of 635, 645 and 920 mg./m². The 2-phenyl benzimidazole was replaced by N-dodecylamino-purine. A plurality of such photosensitive elements were given identical exposures and then processed in the manner described in Example 1 using the same type of image-receiving element with the following processing composition applied in a layer approximately 0.076 mm thick, the processing composition comprising:

Using the above processing composition as a control, the relative effects of the following compounds were compared at the weight percentages indicated in the following tables:
imidazole
2-methyl imidazole
1-methyl imidazole
1,2-dimethyl imidazole
2-methyl pyrazine
3-methyl pyridazine
4-methyl pyrimidine

The following tables show the effects of the test compounds upon the final maximum red, green and blue reflection densities as measured in the neutral column:

The relative rates of transfer of the image dyes was also measured using the same components and measured the density as a function of time using an automatic recording densitometer. The following table indicates the difference in density at the given times between the control and the test compound at 1 and 2% weight per cent, decreased density at a given time being indicated by a minus sign.

It will be seen from the expermental comparisons given above that incorporation of the diazoles or diazines within the scope of this invention are useful to increase the rate of transfer of one or more of the dye developers, particularly in the first minute or two, even though the final density may not be greater. In contrast, such closely related diazoles as imidazoles and 2-methyl imidazole reduced transfer rates and substantially reduced final image densities.

The above examples illustrate how the diazoles and diazines within the scope of this invention may be utilized to modify the sensitometry in desirable aspects.

In the above examples the neutralizing and timing layers were positioned between the image-receiving layer and its transparent support. In certain embodiments it is advantageous to position the neutralizing and timing layer in the photosensitive element, i.e., between the cyan dye developer layer and the opaque support, in the manner described in U.S. Patent No. 3,573,043 issued March 30, 1971 to Edwin H. Land.

In the preferred embodiments the diazole is dissolved in the processing composition. The concentration of the diazole most appropriate for a given film unit may be determined by routine experimentation. In general, if the diazole is in the processing composition, the concentration may be in the range of about 0.5 to 3% by weight; higher concentrations may be used but have not been found to offer any advantages. The preferred concentration is about 0.5 to 1%.

It will be understood that the diazoles also may be used in dye developer color transfer processes wherein the image-receiving element is separated from the developed photosensitive element.

In certain instances the diazole, e.g., 1-methyl imidazole, may exhibit a tendency to photolyze and stain the image. Increasing the coverage of the polymeric acid neutralizing layer and/or placing it in the photosensitive element, has been found to substantially prevent such photolysis under typical normal conditions of use.

In a particularly useful embodiment of this invention, N-n-dodecylamino purine is incorporated in one or more of the dye developer layers. This combination together with some of the diazoles, e.g., 1-methyl imidazole, has been found to give an increase in red speed.

It will be recognized that it is desirable that the dye developers thransfer as rapidly as possible. Efforts have therefore been made to increase the dye transfer rate by the addition of various chemicals, including chemicals which may be considered to be solvents for the dyes. While many compounds may increase the rate of transfer of unoxidized dye developer, few compounds will do this without also increasing the solubility and diffusibility of oxidized dye developer, i.e., dye developer which should be immobilized where development occurred. Such an increase in the diffusibility of oxidized dye developer is undesirable as it will result in unwanted dye transfer producing an increase in minimum density. This is a particular disadvantage in integral positive-negative reflection prints of the type described in the above-mentioned U.S. Patent 3,415,644, since the processing composition is retained in the film and the "solvent" has an extended opportunity to cause unwanted dye transfer.

## Claims

1. A diffusion transfer film unit comprising a photosensitive element comprising a support carrying at least one photosensitive silver halide emulsion layer, each said silver halide emulsion layer having associated therewith a dye developer; an aqueous alkaline processing compostion; an image-receiving layer in superposed or superposable relationship with said silver halide emulsion layer(s) characterized in that said film unit includes a 5- or 6-membered aromatic unsaturated hetero or diazine, cyclic diazole respectively, free of imino nitrogen atoms, said diazole or diazine being a liquid at room temperature.

2. A diffusion transfer film unit according to claim 1 wherein said photosensitive element includes a red-sensitive silver halide emulsion, a green-sensitive silver halide emulsion and a blue-sensitive silver halide emulsion, said silver halide emulsions having associated therewith, respectively, a cyan dye developer, a magenta dye developer and a yellow dye developer.

3. A diffusion transfer film unit according to claim 1 or 2 wherein said image-receiving layer is carried on a second, transparent support.

4. A diffusion transfer film unit according to any one of claims 1-3 wherein said diazole or diazine is initially present in said processing composition.

5. A diffusion transfer film unit according to any of the preceeding claims wherein said diazole or diazine is 1-methyl imidazole, 1,2-dimethyl imidazole, 2-methyl pyrazine, 3-methyl pyridazine, or 4-methyl pyrimidine.

6. A diffusion transfer film unit according to any preceeding claim wherein the concentration of said diazole or diazine is about 0.5 to 3% by weight, preferably about 0.5 to 1%.

7. A diffusion transfer film unit according to any preceeding claim wherein said dye developer is: or

8. A diffusion transfer color process comprising exposing a photosensitive silver halide emulsion, and applying a processing composition to said exposed silver halide emulsion to effect development of exposed silver halide and an imagewise distribution of unoxidized dye developer is formed in undeveloped areas of said silver halide emulsion as a function of said development, said process including the step of transferring by diffusion at least a portion of said imagewise distribution of unoxidized dye developer to an image-receiving layer in superposed relationship with said silver halide emulsion, thereby providing a positive diffusion transfer dye image, characterized in that said process is performed in the presence of a 5- or 6-membered aromatic unsaturated heterocyclic diazole or diazine, respectively, free of imino nitrogen atoms, said diazole or diazine being a liquid at room temperature.

9. A diffusion transfer process according to claim 8 wherein said diazole or diazine is initially present in said processing composition.

10. A diffusion transfer process according to claim 8 or 9 wherein said diazole or diazine is 1-methyl imidazole, 1,2-dimethyl imidazole, 2-methyl pyrazine, 3-methyl pyridazine, or 4-methyl pyrimidine.

11. A diffusion transfer color process according to any of claims 8-11 wherein said diffusion transfer image is a multicolor image.

## Revendications

1. Pellicule complète pour la photographie par diffusion-transfert comprenant un élément photosensible constitué par un support sur lequel sont déposées au moins une couche d'émulsion photosensible à l'halogénure d'argent, chacune desdites couches d'émulsion à l'halogénure d'argent ayant associée à elle un développature chromogène; une composition alcaline aqueuse de traitement; une couche réceptrice d'image superposée ou superposables à ladite ou auxdites couche(s) d'émulsion à l'halogénure d'argent, caractérisée par le fait que ladite pellicule complète renferme un diazole ou une diazine hétérocyclique, aromatique, insaturé, à 5 ou chaînons, respectivement exempt d'atomes d'azote inmino, ledit diazole ou ladite diazine étant un liquide à la température ambiante.

2. Pellicule complète pour la photographie par diffusion-transfert selon la revendication 1, dans laquelle ledit élément photosensible comprend une émulsion à l'halogénure d'argent sensible au rouge, une émulsion à l'halogénure d'argent sensible au vert, et une émulsion à l'halogénure d'argent sensible au bleu, lesdites émulsions à l'halogénure d'argent ayant associés à elles, respectivement, un développateur chromogène cyan, un développateur chromogène magenta et un développateur chromogène jaune.

3. Pellicule complète pour la photographie par diffusion-transfert selon les revendications 1 ou 2, dans laquelle ladite couche réceptrice'd'image est déposée sur un second support transparent.

4. Pellicule complète pour la photographie par diffusion-transfert selon l'une quelconque des revendications 1 à 3, dans laquelle ledit diazole ou ladite diazine est initialement présent(e) dans ladite composition de traitement.

5. Pellicule complète pour la photographie par diffusion-transfert selon l'une quelconque des revendications précédentes, dans laquelles ledit diazole ou ladite diazine est le le 1-méthyl-imidazole, le 1,2-diméthyl-imidazole, la 2-méthylpyrazine, 1 a 3-méthylpyridazine ou la 4-méthylpyrimidine.

6. Pellicule complète pour la photographie par diffusion-transfert selon l'une quelconque des revendications précédentes, dans laquelle la concentration dudit diazole ou de ladite diazine est d'environ 0,5 à 3% en poids, de préférence d'environ 0,5 à 1%.

7. Pellicule complète pour la photographie par diffusion-transfert selon l'une quelconque des revendications précédentes, dans laquelle ledit développateur chromogène est: oder

8. Procédé en couleurs de diffusion-transfert comprenant l'exposition d'une emulsion à l'halogenure d'argent photosensible et l'application d'une composition de traitement sur ladite émulsion à l'halogenure d'argent exposée pour développer l'halogenure d'argent exposé, une distribution selon une image de developpateur chromogène non oxydé étant formée dans les zones non développées de ladite émulsion à l'halogenure d'argent en fonction dudit développement, ledit procédé comprenant le stade de transfert par diffusion d'au moins une partie de ladite distribution selon une image de developpateur chromogène non oxydé sur une couche réceptrice d'image superposée à ladite émulsion à l'halogenure d'argent, fournissant ainsi une image en couleurs positive de diffusion-transfert, caracterisé par le fait que ledit procédé est effectué en présence d'un diazole ou d'une diazine hétérocyclique, insaturée, aromatique, à 5 ou 6 chaînons réspectivement, exempt(e) d'atomes d'azote imino, ledit diazole ou ladite diazine étant un liquide à la température ambiante.

9. Procédé de diffusion-transfert selon la révedication 8 dans lequel ledit diazole ou ladite diazine est initialement present(e) dans ladite composition de traitement.

10. Procédé de diffusion-transfert selon les révendications 8 ou 9 dans lequel ledit diazole ou ladite diazine est le 1-methylimidazole, le 1,2-diméthylimidazole, la 2-méthylpyrazine, la 3-méthylpyridazine ou la 4-méthylpyrimidine.

11. Procédé en couleurs de diffusion-transfert selon l'une quelconque des revendications 8 à 10, caracterisé par le fait que ladite image de diffusion-transfert est une image polychrome.

## Patentansprüche

1. Diffusionsübertragungs-Filmeinheit, enthaltend ein lichtempfindliches Element mit einer Unterlage, die mindestens eine lichtempfindliche Silberhalogenid-Emulsionsschicht trägt, wobei jeder Silverhalogenid-Emulsionsschicht ein Entwicklerfarbstoff zugeordnet ist; eine wäßrig-alkalische Entwicklermasse; eine Bildempfangsschicht, die über der (den) Silberhalogenid-Emulsionsschicht(en) liegt oder darüber gelegt werden kann; dadurch gekennzeichnet, daß die Filmeinheit ein 5- oder 6- gliedriges aromatisches ungesättigtes heterocyclisches Diazol, bezw. Diazin enthält, das frei von Imino-Stickstoffatomen ist, wobei das Diazol oder Diazin bei Raumtemperatur eine Flüssigkeit ist.

2. Diffusionsübertragungs-Filmeinheit nach Anspruch 1, worin das lichtempfindliche Element eine rotempfindliche Silberhalogenid-Emulsion, eine grünempfindliche Silberhalogenid-Emulsion und eine blauempfindliche Silberhalogenidemulsion enthält, wobei diesen Silberhalogenid-Emulsionen jeweils ein balugrüner Entwicklerfarbstoff, ein purpurner Entwicklerfarbstoff und ein gelber Entwicklerfarbstoff zugeordnet ist.

3. Diffusionsübertragungs-Filmeinheit nach Anspruch 1 oder 2, worin die Bildempfangsschicht auf einer zweiten, durchsichtigen Unterlage aufgebracht ist.

4. Diffusionsübertragungs-Filmeinheit nach einem der Ansprüche 1 bis 3, worin das Diazol oder Diazin ursprünglich in der Entwicklermasse vorhanden ist.

5. Diffusionsübertragungs-Filmeinheit nach einem der vorhergehenden Ansprüche, worin das Diazol oder Diazin 1-Methylimidazol, 1,2-Dimethyiimidazoi, 2-Methylpyrazin, 3-Methylpyridazin oder 4-Methylpyrimidin ist.

6. Diffusionsübertragungs-Filmeinheit nach einem der vorhergehenden Ansprüche, worin die Konzentration des Diazols oder Diazins etwa 0,5 bis 3 Gew.-%, vorsugsweise etwa 0,5 bis 1 % beträgt.

7. Diffusionsübertragungs-Filmeinheit nach einem der vorhergehenden Ansprüche, worin der Entwicklerfarbstoff ist: ou

8. Farbdiffusionsübertragungsverfahren, bei dem eine lichtempfindliche Silberhalogenid-Emulsion belichtet und eine Entwicklermasse auf die belichtete Silberhalogenid-Emulsion aufgebracht wird, um die Entwicklung des belichteten Silberhalogenids zu bewirken, und wobei eine bildmäßige Verteilung von nicht oxidiertem Entwicklerfarbstoff in den unentwickelten Bereichen der Silberhalogenid-Emulsion als Funktion der Entwicklung gebildet wird, wobei das Verfahren die Stufe der Diffusionsübertragung mindestens eines Teils der bildmäßigen Verteilung des nicht oxidierten Entwicklerfarbstoffs auf eine Bildempfangsschicht, die über der Silberhalogenid-Emulsion liegt, umfaßt, wodurch ein positives Farbdiffusions-Übertragungsbild erhalten wird, dadurch gekennzeichnet, daß das Verfahren in Gegenwart eines 5- oder 6- gliedrigen aromatischen ungesättigten heterocyclischen Daizols bzw. Diazins, das frei von Imino-Stickstoffatomen ist, durchgeführt wird, wobei das Diazol oder Diazin bei Raumtemperatur eine Flüissigkeit ist.

9. Diffusionsübertragungsverfahren nach Anspruch 8, worin das Diazol oder Diazin ursprüngliche in der Entwicklermasse vorhanden ist.

10. Diffusionsübertragungsverfahren nach Anspruch 8 oder 9, worin das Diazol oder Diazin 1-Methylimidazol, 1,2-Dimethylimidazol, 2-Methylpyrazin, 3-Methylpyridazin oder 4-Methylpyrimidin ist.

11. Farbdiffusionsübertragsungsverfahren nach einem der Ansprüche 8 bis 10, worin das Diffusionsübertragungsbild ein mehrfarbiges Bild ist.
